

June 1, 1937.

J. C. RAH

2,082,027

ELECTRIC DEVICE AND PROCESS OF MAKING THE SAME

Filed Aug. 30, 1933

Fig. 1.



27

Inventor:  
Joseph C. Rah  
By Manufacturer: Bortleas - Dremer  
Attr.:

## UNITED STATES PATENT OFFICE

2,082,027

ELECTRIC DEVICE AND PROCESS OF MAK-  
ING THE SAME

Joseph C. Rah, Chicago, Ill., assignor to The  
Delta-Star Electric Company, Chicago, Ill., a  
corporation of Illinois

Application August 30, 1933, Serial No. 687,457

7 Claims. (Cl. 18—59)

In the pending application of Elias S. Cornell, Charles A. Koerner, and Joseph A. Stoos, Serial No. 685,048, filed August 14, 1933, there is shown a transfer stud which is used on a circuit breaker in connection with other apparatus for effecting a selective connection between one pole of the breaker and either one of two sets of contacts. The present invention is concerned with the construction and method of insulating the transfer stud.

The transfer stud consists, in its essence, of a pair of spaced switch terminals joined by a conducting bar and enclosed, except for the contacting ends of the terminals, in a body of insulation which is molded around the same. The insulation preferably comprises a phenol condensation production known as "bakelite".

In the design of a stud of this type, primary consideration must be given to two important problems arising from the nature and use of such a device. Firstly, the mechanical problems which arise in connection with the application of insulating materials to an electrical conductor in order to effect a perfect and permanent adhesion therebetween and yet to provide sufficient elasticity throughout the life of the device to eliminate the destructive effect of the differences in coefficient of expansion of the various materials, must be overcome by proper selection, design and application of the materials. Secondly, the electrical problems which are involved in properly proportioning the various materials used in insulation, as such materials have different dielectric constants. In connection with this latter feature, for example, these materials must be so selected and proportioned that the entire assembly will withstand operating potentials running as high as 15,000 volts, and testing potentials running up to approximately 40,000 volts. Also, the design must be such that the maximum voltage gradient at any point in the insulating structure will be below the limit at which corona will form, since formation of corona discharges within the insulating structure will ultimately cause breakdown of the insulation. With these primary considerations in mind, the present invention is directed particularly to the provision of a terminal stud in which these problems have been adequately solved.

When plastic material, such as "bakelite" or the like, is molded around a solid conductor, difficulties are encountered due to the unequal expansion and contraction of the molded material and the conductor under thermal changes. This causes cracking of the molded material. It is

an object of the present invention to overcome this difficulty. I propose to accomplish this result by coating the conductor with an elastic material, such as gum rubber, and molding the "bakelite" insulation around the coated conductor. By this arrangement the rubber constitutes a floating support for the conductor within its molded insulation and allows for relative expansion and contraction between the conductor and the molded insulation under thermal changes.

The gum rubber is far inferior to the molded material as an electric insulator, and it is not relied upon for that purpose. The molded insulation is made of a thickness necessary to supply the requisite insulation. When plastic "bakelite" is formed around rubber there is a tendency for the rubber to penetrate into the "bakelite" under the heat and pressure prevailing during the molding process. The rubber tends to form needle-like projections extending into the body of the "bakelite". Since the insulating properties of the rubber of each needle-like projection are far inferior to the insulating properties of the "bakelite" which it replaces, the net result of the formation of these projections is a reduction in the insulation afforded by the molded "bakelite". This reduction is proportionate to the extent of penetration or length of the longest projection, since the insulation of the entire piece is no greater than the insulation at the weakest part thereof. It is one of the objects of the present invention to prevent the penetration of the rubber into the "bakelite" during the molding process.

I have found that the outer surface or skin of a body of rubber may be made tougher than the main body of rubber. This tough skin tends to resist the tendency of the main body of rubber to flow into the plastic material under the pressure and temperature conditions prevailing during molding. However this skin is so thin that, while it resists the tendency to penetrate, it can not prevent it. To overcome this difficulty, I propose to build up the rubber coating on the conductor in the form of a large number of very thin layers, each layer of which is treated to form a tough skin thereon before the next thin layer of rubber is applied. By this method I build up the rubber to the requisite thickness and of qualities such that it does not penetrate the molded material during the molding stage. However, it is to be noted that the rubber is not hardened or vulcanized by this process, as the use of a vulcanized rubber is undesirable, since it has a pronounced tendency to disintegrate due

to the effect of corona discharges, and the uniformity of its dielectric characteristic is thus disturbed. On the other hand, the use of a softer, unvulcanized rubber as employed in the 5 present invention eliminates, to a great extent, any initial or subsequent formation of air pockets or voids, thus reducing the possibility of corona and its resulting destructive effects.

Another object of the present invention is to 10 prevent, as far as possible, any incipient corona, since if corona discharges are once allowed to be set up, their subsequent effect is cumulative, resulting in untimely breaking down of the insulation.

15 The attainment of the above and further objects of the present invention will be apparent from the following specification taken in conjunction with the accompanying drawing forming a part thereof.

20 Figure 1 is a view, in partial section, showing my improved transfer stud as part of an adapter which is mounted on the head of a circuit breaker; and

25 Figure 2 is a top view, in reduced scale, of the transfer stud.

Reference may now be had more particularly to Figure 1. For the purpose of illustration, I have shown at 1 a portion of the head of an oil circuit breaker. The circuit breaker includes a 30 socket terminal 2 for establishing electrical connections to one side of the breaker, and a terminal stud 3 for establishing connections to the other side of the breaker. The socket terminal 2 is of a construction such as shown in the pending application of Alfred Alsaker and Fred H. Cole, Serial No. 681,158, filed July 19, 1933.

Briefly, the socket terminal comprises a large number of contact wires 4, swaged or otherwise suitably secured to a plug 5 that is threaded 40 over a terminal stud 6 comprising one terminal of the circuit breaker. Coiled springs 7, in the form of rings, embrace the contact wire assembly and urge the wires inwardly into firm engagement with a contact plug that is receivable by the socket terminal. A plurality of internal rings 8 limit the extent of inward collapse of the contact wires when the socket does not contain a plug. A sleeve 9, of suitable insulation, surrounds the contact socket for preventing accidental engagement therewith.

It is to be noted that the terminal stud 3 is appreciably below the terminal stud 6. When the adapter, to be presently described, is mounted in place it brings the overall height of the corresponding terminal of the circuit breaker to that of the socket terminal 2.

The adapter comprises a transfer stud 10 and a transfer plug. The transfer stud includes a copper bar 12, one end of which is secured to 60 the stud 3. The other end of the copper bar carries a stud 13 that threads into a plug 15. The stud 3, which threads through the copper bar 12, also threads into the base of a copper plug 14. The copper bar 12 is covered with a layer 65 of rubber 16, in a manner to be more fully set forth as the description proceeds, and is enclosed in a body of insulation 17 which is molded around it and may comprise any suitable insulation, such as the material known as "bakelite".

70 The body of insulation includes cylindrical pockets 18 and 19 formed integrally with the body of insulation 17. The ends of the copper bar 12 extend into the cylindrical pockets and divide each of these pockets into upper and lower cylindrical portions. The transfer stud includes

a supporting leg comprising an insulating rod 20 and an insulating tubing 21, and a mounting base 22. The rod 20 is secured in place by the stud 13, the lower end of which threads into the rod. The mounting base is secured to the rod 20 by means of a bolt 23 that threads into the rod 20 and holds the base thereto. The mounting base 22 is adapted to be bolted or otherwise secured to the head of the circuit breaker 1.

The base of each of the contact plugs 14 and 15 is internally threaded for receiving the studs 3 and 13 respectively, as previously set forth. The stud 3 establishes the electric circuit between the circuit breaker and the copper bar 12, and also establishes a circuit to the plug 14. The stud 13 extends the electric circuit between the bar 12 and the plug 15. Tubes of insulation 24 and 25 are internally threaded at their lower ends and thread over the external thread on the bases of the plugs 14 and 15 respectively. 20 These tubes are spaced from the plugs by an amount sufficient to permit the entry of a socket terminal of a transfer plug.

The transfer plug is indicated at 30. It comprises a unitary body of insulation 31 including a bridge member 32 having a cap 33 formed at one end thereof and a socket receiving cylindrical formation 34 at the opposite end. A pair of oppositely facing sockets 35 and 36, of a construction similar to the socket terminal 2, are 30 secured to the portion 34 of the transfer plug. A tube of insulation 37 surrounds the socket 35, being fitted over a cylindrical portion of the main body of insulation comprising the transfer plug. A pair of spring clips 40-41, carried by the transfer stud extend through a centrally located opening in the bridge portion 32 of the transfer plug and serve to snap the transfer plug into its fully closed position when it is brought approximately to its fully closed position.

The springs 40-41 are suitably secured to the opposite sides of an upwardly extending portion 42 of insulation formed integrally with the body of insulation 17. In order to strengthen the body of insulation 42 the copper bar 12 is provided with a hole 43 immediately beneath the body of insulation 42. During the molding process the hole 43 is, of course, filled with insulation which constitutes an integral part of the insulation 17. The insulation within this hole thus serves to take 50 some of the stress imposed upon the main body of insulation 17 and prevents an overstressing of the comparatively thin insulation between the bar 12 and the outer surface of the body 17.

In the position shown in Figure 1 the transfer 55 plug covers the plug 14, the socket 36 being in a position to engage the plug 15. This places the socket 35 at a given distance from the socket terminal 2. If desired, the transfer plug may be reversed so that the cap 33 covers the plug 60 15, and the socket 36 engages the plug 14. When this is done, the socket 35 is closer to the socket terminal 2 than when it is in the position indicated in Figure 1. In its two alternate positions, the socket 35 is adapted to engage different plugs 65 for establishing different circuits. It is to be noted that in either position of the plug all of the live parts of the transfer stud are fully enclosed by adequate insulation.

An explanation will now be given of the mode 70 of forming the insulation around the copper bar 13. The copper bar is first freed of all sharp corners and projections, all of the corners being rounded, and is then thoroughly cleaned. The bar is then dipped into a vat containing pure 75

gum rubber dissolved in benzine and to which a plasticizer has been added to retard vulcanization. The plasticizer may comprise any suitable oil which will withstand a temperature of about 300° F. The first coat is dried in a drying oven for about one-half hour at a temperature of about 140° to 150° F. The bar is then taken out of the oven and permitted to cool at room temperature and is again dipped into the vat and 5 again baked, this being repeated about five or six times until the desired thickness of rubber has been built up. I have found that a thickness of about  $\frac{1}{2}$  of an inch is sufficient. The last coat of rubber is baked for approximately two 10 hours, after which it is gradually cooled to room temperature over a period of about twelve hours. This results in a thorough drying of the rubber. At the same time, since the rubber is not heated to its vulcanizing temperature, this 15 rubber coating remains in a soft, plastic and unvulcanized state, whereby it is effective for accommodating the differences in expansion between the various materials, and at the same time eliminates, to a great extent, any formation 20 of voids or air pockets, and thus reduces the possibility of incipient corona discharges. The bar, with its rubber coating, is then placed in a "bakelite" mold to form a "bakelite" enclosure for the 25 bar. It is cured by baking for ten to fifteen minutes at 350° F. It is then aged outside of the mold by baking for approximately forty eight hours at 300° F. Thereafter it is coated with "bakelite" resin varnish, and the insulating rod 30 and the insulating tubing 21, both also coated 35 with the "bakelite" resin varnish, assembled in place. This assembly is then baked for four to six hours at 275° F. The length of this period of baking is determined by the time required to produce a high surface resistance, as determined 40 by proper electrical tests.

The ageing outside of the mold for forty eight hours is for the purpose of causing the "bakelite" to shrink all that it will ever shrink. This assures that there will be no shrinkage of the "bakelite" during the life of the device. This 45 overcomes the difficulty due to the tendency of "bakelite" to shrink as it ages, since such shrinkage may cause cracking of the "bakelite", to the detriment of the device in service. By artificially 50 ageing the "bakelite" I produce, in forty eight hours, all the shrinking that would normally take place during the entire life of the device. Those devices that crack during the ageing process can be rejected, thus assuring that the serviceable 55 devices will remain serviceable during the life of the device.

When plastic "bakelite" is formed around a rubberized compound, there is a tendency for the rubber to penetrate into the "bakelite" in the 60 form of needle-like projections extending into the body of the "bakelite". Since the rubber has poor insulating qualities, and is not relied upon for insulation, such penetration will reduce the insulating properties of the "bakelite" 65 to a substantial amount and must, therefore, be prevented. By applying the rubber onto the copper bar in a number of very thin coats, the plasticizer forms a continuous surface around each layer and avoids the production of a spongy mass 70 of rubber. The plasticizer, it appears, strengthens the outer coating of each layer and, by surface tension, serves to hold the rubber against penetrating into the "bakelite" under the action 75 of the heat and pressure incident to the molding operation.

In compliance with the requirements of the patent statutes I have herein shown and described a preferred embodiment of my invention. It is, however, to be understood that the invention is not limited to the precise structure and method described, the same being merely illustrative of the principles of the invention. 5

What I consider new and desire to secure by Letters Patent is:

1. The method of insulating an electrical conductor carrying substantial current and subjected to expansion due to heating by said current, which comprises superposing a plurality of enveloping layers of a solution of gum rubber and a plasticizer about said conductor, baking each of 10 said layers at a temperature below the vulcanizing temperature of said rubber before application of the next succeeding layer, and enclosing said layers in a hard phenol condensation product casing by molding said casing thereabout 15 under heat and pressure. 20

2. The method of enclosing an electrical conductor carrying substantial current and subjected to expansion due to heating by said current, within a hard molded insulating casing of high 25 dielectric strength and of a different coefficient of expansion than that of said conductor, which comprises applying a plurality of successive layers of a solution consisting of gum rubber and a plasticizer about said conductor, drying each 30 layer of said solution prior to application of the next succeeding layer at a temperature below the hardening temperature of said rubber, and molding a phenol condensation product about said 35 plurality of layers by application of heat and pressure, said layers being sufficiently plastic to accommodate relative movement between said conductor and said molded insulation.

3. An article of manufacture comprising an 40 electrical conductor for carrying relatively high potentials and subjected to longitudinal expansion due to the heating effects of the current in said conductor, a plurality of layers of plastic rubber enveloping the lateral and end surfaces of said conductor, said rubber including a plasticizer 45 for preventing the same from hardening and providing a strengthened skin surface for each of said layers, and a molded phenol condensation product enclosing the outermost one of said layers and having a relatively low coefficient 50 of expansion, said plastic layers being resilient to provide for relative movement between said conductor and said molded condensation product.

4. The method of insulating an electrical conductor at relatively high potentials and subjected to expansion due to the heating effects of the current in said conductor, which comprises enclosing said conductor in a plastic envelope of 60 adhering rubber, said rubber having a plasticizer incorporated therein for retaining it in a plastic condition and providing a strengthened outer 65 skin surface, applying an insulating casing thereover comprising a molded phenol condensation product having a relatively low coefficient of expansion as compared to said conductor, said intermediate rubber envelope accommodating relative movement between said conductor and said casing, and ageing said insulating casing to remove shrinking stresses therefrom.

5. The method of insulating an electrical conductor carrying current at relatively high potentials and subjected to expansion due to the heating effects of said current which comprises applying a series of layers of a solution consisting 70 of gum rubber and a plasticizer about the con- 75

ductor, applying an outer enclosing coating of a moulded phenol condensation product about said series of layers, and proportioning the relative thicknesses of the insulating coatings to produce a maximum voltage gradient for each insulating coating which will be below a value at which corona forms when the conductor is subjected to a definite operating voltage.

6. A transfer stud comprising a solid metallic conductor, a buffer comprising a plurality of substantially homogeneous layers of unvulcanized gum rubber disposed over said conductor, a body of insulation comprising a phenol condensation product molded around the conductor and buffer, said buffer being yielding to provide for relative movement between said conductor and said body of insulation, the outer surface of said rubber being toughened to prevent relative

impregnation between said insulation and said rubber, and switch terminals at the opposite ends of the conductor.

7. The method of insulating an electric conductor subject to current sufficient to cause expansion thereof by heating, which comprises successively applying enclosing layers of gum rubber and a plasticizer solution over said conductor, baking each layer at a temperature below the vulcanizing temperature of said rubber before application of the next succeeding layer, molding an insulation body comprising a condensation product about the outermost layer of said rubber, and hardening said insulation body by heat and pressure to produce a substantially rigid body over said rubber.

JOSEPH C. RAH.